

# UNITED STATES PATENT OFFICE.

CLEMENT L. PERKINS, OF PITTSBURGH, PENNSYLVANIA, ASSIGNOR TO METALS RECOVERY COMPANY, OF NEW YORK, N. Y., A CORPORATION OF MAINE.

## FLOTATION OF MINERALS.

1,364,304.

Specification of Letters Patent.

Patented Jan. 4, 1921.

No Drawing.

Application filed July 21, 1919. Serial No. 312,247.

To all whom it may concern:

Be it known that I, CLEMENT L. PERKINS, a citizen of the United States, residing at Pittsburgh, in the county of Allegheny, 5 State of Pennsylvania, have invented certain new and useful Improvements in Flotation of Minerals; and I do hereby declare the following to be a full, clear, and exact description of the invention, such as will 10 enable others skilled in the art to which it appertains to make and use the same.

This invention relates to the concentration of minerals, such as sulfid ores and the like, by flotation, and is based upon the discovery that improved results can be obtained by carrying out the flotation operation with the addition, to the ore or mineral pulp, of certain non-oleaginous solid organic compounds, which themselves have 15 substantially no frothing properties, but which have valuable properties as collecting agents for the mineral. Such collecting agents, although substantially non-frothing, nevertheless so act upon the minerals that 20 they very materially assist in the recovery of the minerals when used in connection with a suitable frothing agent.

Among the agents which are of particular value as collecting agents, and which 30 are substantially non-frothing, are reduced compounds which are relatively easily oxidizable, such as, for example, diazo-amino-benzene. It may be that these compounds are adsorbed at the surface of the sulfid or 35 mineral particles, and that they so modify the sulfid or mineral surfaces that these surfaces are less easily wet by water or made more readily susceptible to attachment by the air bubbles. In some cases the reduced 40 compound is apparently further reduced by the action of the sulfid particles, so that the action may partake of both a chemical and physical nature. These agents also appear to be adsorbed to some extent by certain of 45 the gangue particles, but in this case oxidation of the collecting agent apparently takes place at the surface of the gangue particles, so that the actual surface presented is an oxidizing or oxidized surface,

while in the case of the sulfid particles it 50 appears to be a reduced surface. However, I do not desire to limit myself by any theoretical explanation of the mechanism of the action of these collecting agents.

Although the collecting agents are substantially insoluble, and are commonly referred to as insoluble, nevertheless, they are soluble to a very small degree, and it appears to be by reason of this solubility that they are able to act upon the minerals and 60 exert their marked selective and collecting properties.

These collecting agents are, as above noted, non-frothing, and it is, therefore, important to supplement their action by an 65 agent which will provide an appropriate amount of froth. The frothing agent, however, may be entirely inadequate to perform the flotation process by itself, inasmuch as its function appears to be simply to provide 70 bubbles in sufficient quantity and of sufficient persistency to overflow into the launder of the flotation machine, thereby mechanically facilitating the removal of the mineral concentrate.

Among the collecting agents of the character above referred to, that is, which are substantially non-frothing, are included certain of the aromatic thio-ureas, and many of the azo and diazo compounds. A collecting agent which I have found of particular value is diazo-amino-benzene,



The collecting agents can be incorporated 85 with the ore or mineral pulp in any suitable manner which will insure their uniform incorporation and dissemination throughout the pulp. They may thus be incorporated by grinding in the tube mill in which 90 the ore itself is ground, or they may be dissolved in an organic solvent therefor, and the resulting solution added to the ore pulp. When a solvent of the collecting agent is employed, it may advantageously itself be 95 an agent with good frothing properties, so that its action will supplement the collecting action of the collecting agent. After

the collecting agent and a suitable frothing agent have been thoroughly and uniformly distributed throughout the ore or mineral pulp, the resulting mixture is subjected to 5 a flotation operation, as in an ordinary Cal-low cell, or in apparatus where the air is incorporated in the ore pulp by mechanical agitation.

It is of advantage in many cases to add 10 to the ore pulp a small amount of alkali, which may be sufficient in amount to give to the ore pulp a distinct alkaline reaction. When alkalis are used, it is desirable to give them an appreciable time of contact 15 with the ore pulp before subjecting the latter to flotation. When possible, it appears preferable to add the alkalis in the grinding mill, so that they will be present during the grinding operation. The alkali 20 may be caustic alkali, such as sodium hydrate, or an alkaline salt, such as sodium carbonate, or even lime or calcium oxid or hydrate can be used.

The amount of the collecting agent added 25 may vary somewhat, and may be as little as one-fifth or one-fourth of a pound per ton of ore (that is, calculated on the weight of the ore and not of the ore pulp). I have obtained good results with the use of as little as one-thirtieth of a pound per ton of ore. Larger amounts may, however, be used.

The invention will be further illustrated by the following specific examples of tests 35 made upon a copper sulfid ore having a silicious gangue containing its floatable or sulfid copper in the form of a mixture of chalcocite and chalcopyrite, that is, so-called porphyry ores, such as those of the Utah 40 Copper Company. In general, treatment of the ore with alkalis, as above noted, gives improved results, the alkalis themselves apparently having a valuable effect upon the ores in improving the floatation thereof.

45 1. *Diazo-amino-benzene and terpineol.*— 500 parts by weight of Utah Copper Company's ore was ground in the pebble mill with 250 parts of water, sodium hydroxid equivalent to two pounds per ton of dry 50 ore, and diazo-amino-benzene equivalent to one-fifth pound per ton. The ground pulp was transferred to a Cal-low rougher cell, diluted, and floated with the addition of terpineol equivalent to about one-tenth 55 pound per ton. The heads for this test contained 1.42 per cent. copper, the concentrates produced contained about 22.4 per cent. copper, and the recovery was about 91.4 per cent.

60 2. *Diazo-amino-benzene and terpineol.*— The details of the test were the same as those of No. 1, except that the proportion of diazo-amino-benzene was reduced to one-thirtieth pound per ton. The heads for 65 test No. 2 contained 1.38 per cent. copper,

the concentrate produced contained about 17.3 per cent. copper, and the recovery was about 87.7 per cent.

3. *Diazo-amino-benzene and pine oil.*— The details of this test were the same as 70 those of No. 1, except that steam-distilled pine oil was substituted for terpineol. The proportion of pine oil used was about one-fourth pound per ton of dry ore. The heads for test No. 3 contained 1.39 per cent. 75 copper, the concentrates produced contained about 17.9 per cent. copper, and the recovery was about 88.6 per cent.

4. *Diazo-amino-benzene dissolved in xylidin.*—Five hundred parts by weight of 80 Utah Copper Company's ore were ground with 250 parts of water and sodium hydroxid equivalent to two pounds per ton of dry ore. The ground ore pulp was diluted, and to the ground and diluted pulp 85 was then added a solution of diazo-amino-benzene in xylidin. The proportion of the compound reagent used was one-half pound per ton of dry ore. It contained about 80 per cent. xylidin and 20 per cent. diazo-amino-benzene. The pulp was transferred immediately to a Cal-low rougher cell and floated. The heads for this test contained 1.39 per cent. copper, the concentrates contained about 21.9 per cent. copper, and the 90 recovery was about 91.2 per cent.

As appears from these examples, different frothing agents may be used, and the collecting agents may be itself dissolved in a solvent which has good frothing qualities. Xylidin is a good example of a valuable floatation agent which serves as a solvent for the diazo-amino-benzene and supplies the necessary froth for the floatation operation. Among other solvents may be 100 mentioned anilin, dimethyl anilin, toluidin and other organic liquids in which the particular collecting agent is soluble, such as cresol, alcohol, etc. The solution of diazo-amino-benzene in xylidin can be promoted 105 by heating, but prolonged heating may result in chemical changes which reduces the effectiveness of the resulting product.

The collecting agent can with advantage be used in addition to many of the usual oil 110 mixtures which are commonly employed in floatation, with resulting improvements in the floatation operation. Flotation oils or oil mixtures which are good frothing agents, such as pine oil and other wood 115 distillation oils, are of particular value, inasmuch as they supplement the action of the collecting agent, and are themselves supplemented in their ore floating properties 120 by the collecting action of the collecting agent.

In the floatation of zinc-lead ores, it has been found of advantage to grind the collecting agent with the neutral ore pulp; and still better results have been obtained when 130

copper sulfate and sulfuric acid were also used in the proportion of about one pound of each per ton of dry ore. A small amount of a suitable frothing agent, as above noted, 5 should also be used.

It is characteristic of the invention that the froth obtained is readily broken up, while a relatively clean concentrate and high recovery can, nevertheless, be obtained.

10 A part of the collecting agent, together with a part of the frothing agent, can sometimes be recovered so that they are available for use in the treatment of further amounts of ore; for example, by recovering 15 the circuit water from the concentrates, or even that from the tailings, and returning the same to the process, with resulting economy in the amount to be added for subsequent operations. The amount of the collecting agent can, however, in many cases 20 be reduced to such a small amount that it is feasible to practise the invention without such recovery of the agents employed.

As above noted, the action of the collecting 25 agent appears to be a selective action upon the mineral surfaces, rather than any action of importance upon the water itself, inasmuch as the removal of all water from the ore pulp, after the collecting agent has 30 been incorporated therewith, and the subsequent washing of the ore, does not deprive it of its improved flotation properties when made into an ore pulp with fresh water and subjected to flotation. Investigations 35 of this kind indicate that the collecting agents have a selective modifying effect upon the mineral surfaces, and that any modifying effect upon the water is incidental. The modifying action of the collecting 40 agents upon the mineral particles is sufficiently marked so that it is possible to raise larger mineral particles, and hence finer grinding becomes of less importance, or unnecessary.

45 The process in which organic nitrogen compounds, including azo and diazo compounds, many of which are non-frothing collecting agents, are employed, is claimed in my companion application, Serial No. 50 312,248 filed of even date herewith; the more specific claims of said application being directed to the process in which diazo-amino compounds are employed, and specifically to the process in which diazo-amino-toluene is 55 employed.

The flotation process in which organic thio-urea and other nitrogen-sulfur compounds, such as thio-carbanilid, many of which are likewise non-frothing collecting 60 agents, are employed, is claimed in two joint applications, of the present applicant with Ralph Sayre Serial No. 284,981, filed March 25, 1919, and Serial No. 337,322, filed November 11, 1919.

65 The more comprehensive claims of the

present case are intended to be of a comprehensive and generic character for the process in which such substantially non-frothing collecting agents are employed; while the specific claims of the present case 70 are directed to the process in which diazo-amino-benzene is employed.

I claim:

1. The method of effecting the concentration of minerals by flotation, which comprises adding to the mineral pulp a small amount of a substantially non-oleaginous organic mineral collecting agent which is substantially non-frothing, and subjecting the resulting mixture to a froth flotation operation; substantially as described. 75

2. The method of effecting the concentration of minerals by flotation, which comprises adding to the mineral pulp a substantially non-frothing, non-oleaginous organic mineral collecting agent which is substantially non-frothing, together with an agent having good frothing properties, and subjecting the resulting mixture to a froth flotation operation; substantially as de- 80 scribed. 85

3. The method of effecting the concentration of minerals by flotation, which comprises adding to the mineral pulp a small amount of a reduced and easily oxidizable organic mineral collecting agent which is substantially non-frothing, and subjecting the resulting mixture to a froth flotation operation; substantially as described. 95

4. The method of effecting the concentration of minerals by flotation, which comprises adding to the mineral pulp a small amount of a reduced and easily oxidizable organic mineral collecting agent which is substantially non-frothing, together with an agent having good frothing properties, and subjecting the resulting mixture to a froth flotation operation; substantially as de- 100 scribed. 105

5. The method of effecting the concentration of minerals by flotation, which comprises adding to the mineral pulp a solution of a substantially non-frothing non-oleaginous organic collecting agent in an organic solvent therefor which has good frothing properties, and subjecting the resulting mixture to a froth flotation operation; substantially as described. 110 115

6. The method of effecting the concentration of minerals by flotation, which comprises adding to the mineral pulp a small amount of a reduced and readily oxidizable organic mineral collecting agent which is substantially non-frothing and which is dissolved in a solvent therefor which is a good frothing agent, and subjecting the resulting mixture to a froth flotation operation; substantially as described. 120 125

7. The method of effecting the concentration of minerals by flotation, which com- 130

4  
prises adding to the mineral pulp a small amount of diazo-amino-benzene, and subjecting the resulting mixture to a froth flotation operation; substantially as described.

8. The method of effecting the concentration of minerals by flotation, which comprises adding to the mineral pulp a small amount of diazo-amino-benzene, together with an agent having good frothing properties, and subjecting the resulting mixture to a froth flotation operation; substantially as described.

9. The method of effecting the concentration of minerals by flotation, which com-

prises adding to the mineral pulp a small amount of diazo-amino benzene, together with a small amount of a frothing oil, such as pine oil, and subjecting the resulting mixture to a froth flotation operation; substantially as described.

10. The method of effecting the concentration of minerals by flotation, which comprises adding to the mineral pulp a small amount of diazo-amino-benzene, dissolved in an organic solvent therefor, and subjecting the resulting mixture to a froth flotation operation; substantially as described.

In testimony whereof I affix my signature.

CLEMENT L. PERKINS.